

## UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MAINE.

## HEELING BOARD.

No Drawing.

Application filed December 21, 1922. Serial No. 608,357.

*To all whom it may concern:*

Be it known that I, ALBERT L. CLAPP, a citizen of the United States, residing at Danvers, in the county of Essex and State 5 of Massachusetts, have invented new and useful Improvements in Heeling Boards, of which the following is a specification.

This invention has for its object the production of a fibrous waterproof board, which 10 may be used for the manufacture of rands, heel boards, and other parts of footwear, as well as for the manufacture of various other articles for use in the arts, by the 15 employment of a paper machine wherein the fibers are felted and sheeted.

A further object of the invention is the utilization of certain waste material resulting from the manufacture of box toes.

In the manufacture of "vulco-box toes" 20 so-called, which are today used in very large quantities in footwear, a fibrous sheet is produced in which is incorporated, usually by saturation or impregnation, such thermo-plastic compounds as bitumens, resins, waxes, 25 drying oils, and certain resinates, in various combinations or mixtures, which impart stiffness and resiliency to the fibrous blank, which soften upon the application of moderate heat so that the blank may be molded 30 about the end of the last in the pulling-over or end-lasting operation, and which set rapidly on being cooled. After the sheet has been formed and saturated or impregnated with the thermo-plastic compound, it 35 is cut into blanks of appropriate size and shape to serve as the box-toe stiffeners, and, as such blanks are irregular, there is of necessity a great waste of the raw sheet material in the form of cuttings or scrap. 40 The thermo-plastic compound in the scrap material is solid at ordinary temperatures such as shoes may be subjected to in wear, and are pulverizable or reducible by grinding.

I have discovered that it is possible to 45 disintegrate the box-toe waste by dry grinding as by the use of an Abbe grinder, and that such an operation may be successfully carried on,—occasionally throwing a small 50 quantity (a handful, for example) of talc into the machine to prevent the thermo-plastic compound from sticking to the blades. The effect of the operation is more or less to separate the felted fibers,—usually 55 wool, cotton, hair, etc.,—and to break up

the thermo-plastic compound, some of which is thereby freed from the fibers. Since these particles of the compound are of great value in the production of a board according to the present invention, some device must be employed for their recovery 60 and use.

I have discovered that tanned leather fibers, when subjected to proper treatment, 65 have the property of entraining or retaining the particles of thermo-plastic compound, in the preparation of an aqueous pulp and its formation in a sheet, and such fibers in addition give to the finished board the 70 appearance of leather, which is highly desirable.

Further I have found that, in securing optimum results in the production of my new fiber board, it is desirable to employ 75 some fluxing agent, which can be incorporated in the aqueous pulp, for fluxing and fusing the thermo-plastic compound originally contained in the box-toe scrap. For this purpose, Montan wax, because of its 80 low viscosity when molten and resultant penetrability, is most desirable.

I shall now give several examples which serve to illustrate my process and my new fiber board.

Example I.—I place in a common beating engine, such as used for preparing pulp for the manufacture of paper or paper felt, 85 20 to 35 parts (by weight) of disintegrated tanned leather scraps or chips, 10 to 15 parts of cellulosic material such as sulphite 90 or sulphate pulp or screenings, manila, mixed papers or rope stock, and 30 to 70 parts of box-toe waste or scraps (the latter having been disintegrated or ground while dry), together with sufficient water to ensure proper circulation of the stock in the beater. The stock is beaten hard for some time, say four to five hours, until it is fairly 95 smooth. (In some cases, the cellulosic material is alone subjected to beating and partial hydration before the leather and the box-toe waste are added and beaten.) I now preferably add to the stock, especially 100 where the proportion of box-toe waste and its contained thermo-plastic compound is 105 relatively small, an amount, say 10 parts, of powdered Montan wax or equivalent fluxing agent, which is thoroughly mixed with the stock. Then a precipitating agent 110 (7 parts of powdered alum for example)

is beaten or brushed by the beaten roll into the pulp, and reacts with certain gelatinous portions of the leather, and forms a gelatinous precipitate which coagulates, and carries down free particles of thermo-plastic compound and the particles of Montan wax, if the latter be employed, and fixes them on the fiber. When the precipitation is complete and the stock is in a fine condition, it is now transferred to the paper machine, and sheeted either in a continuous web by a multi-cylinder machine or in a tube on a wet machine; in which latter case, the tube is slit and stripped from the make-up roll.

Example II.—In this case are used: 35 parts disintegrated tanned leather, 30 parts disintegrated box-toe waste, 15 parts sulphate pulp, 20 parts powdered Montan wax, 20 parts fine hydrated lime, 3 parts rosin size syrup, 2 parts silicate of soda, 7 parts powdered alum.

The lime, leather, box-toe waste and sulphate pulp are thoroughly beaten for some hours, and then the Montan wax, rosin size and silicate of soda are added and thoroughly distributed throughout the mass; whereupon the alum is thoroughly dispersed throughout the pulp, after which the pulp is sheeted on a paper machine. The function of the lime is to precipitate the tannin of the leather and restore the color of the leather to its original hue. The silicate of soda and the rosin size are precipitated by alum as aluminum silicate and aluminum resinate which coagulate and precipitate the free particles of Montan wax and thermo-plastic compound and fix them on the fibers.

Example III.—In this case are used: 20 to 30 parts disintegrated tanned leather, 10 parts sulphate pulp, 70 parts disintegrated box-toe waste, 1 part fine hydrated lime, 2 parts bichromate of soda and/or 1 part sodium carbonate, 5 parts rosin size, 7 parts alum.

Substantially the same procedure is followed as in Example II. The soda ash and/or bichromate of soda are added to the beater coincidently with the lime and the leather, cellulose fiber and box-toe waste. In this case, the function of the bichromate of soda and the carbonate of soda is to react with the tannin and restore to the leather a brown shade. It will be observed that, since a large proportion of box-toe waste is used, I am able to dispense with Montan wax as an ingredient.

The sheeted material, formed on a paper machine from the pulp produced in the foregoing examples, is dried, and is then heated and pressed (as by the use of hot calender rolls) sufficiently to flux the contained thermo-plastic compound and cause its coalescence throughout the sheet, and is thereby

made hard, dense and waterproof. The sheet may now be skived, and the cut surface presents the appearance of leather. Because of the contained gums, resins, etc., the cut edges are capable of receiving and retaining a fine polish.

What I claim is:—

1. A fiber board comprising cellulose fibers, leather fibers, and disintegrated fibrous waste containing a thermo-plastic compound, with the fibers in felted relation and the particles of thermo-plastic compound distributed and precipitated throughout the board.

2. A fiber board comprising cellulose fibers, leather fibers, fibrous waste containing a thermo-plastic compound, and a thermo-plastic compound having a relatively low viscosity when molten, with the fibers in felted relation and the particles of thermo-plastic compounds distributed throughout the board.

3. A hard dense fiber board comprising cellulose fibers, leather fibers and fibrous waste containing a thermo-plastic compound, with the fibers in felted relation and the thermo-plastic compound distributed throughout and coalesced within the board, said board being compacted and presenting, when cut, a surface capable of receiving a polish.

4. A process of producing fiber board, which comprises comminuting fibrous waste containing a thermo-plastic compound, forming such disintegrated waste together with cellulose fibers and leather fibers into an aqueous pulp, and sheeting such pulp with the fibers in felted relation and the thermo-plastic compound distributed throughout the sheet.

5. A process of producing fiber board, which comprises disintegrating box-toe waste containing a thermo-plastic compound, forming such disintegrated waste together with cellulose fibers, leather fibers, and a crushed thermo-plastic compound of low viscosity when molten into an aqueous pulp, and sheeting such pulp on a paper machine.

6. A process of producing fiber board, which comprises disintegrating box-toe waste containing a thermo-plastic compound, forming such disintegrated waste together with cellulose fibers and leather fibers, adding a precipitant to and mixing it in said pulp, and sheeting the pulp on a paper machine.

7. A process of producing fiber board, which comprises disintegrating box-toe waste containing a thermo-plastic compound, forming such disintegrated waste together with cellulose fibers, leather fibers, and a crushed thermo-plastic compound of low viscosity when molten into an aqueous pulp, incorporating in the pulp a material adapted to be precipitated, adding to the pulp a

precipitant for the precipitation thereof, and sheeting the resulting pulp on a paper machine.

8. A process of producing fiber board, which comprises disintegrating box-toe waste containing a thermo-plastic compound, forming such disintegrated waste together with cellulose fibers, leather fibers, and a crushed thermo-plastic compound of low viscosity when molten into an aqueous pulp, incorporating sodium silicate in said pulp, incorporating alum in said pulp for precipitating a gelatinous precipitate, and sheeting said pulp in a paper machine.

9. A process of producing fiber board,

which comprises disintegrating box-toe waste containing a thermo-plastic compound, forming such disintegrated waste together with cellulose fibers, leather fibers, and a crushed thermo-plastic compound of low viscosity when molten into an aqueous pulp, incorporating sodium silicate in said pulp, incorporating alum in said pulp for precipitating a gelatinous precipitate, and sheeting said pulp in a paper machine.

In testimony whereof I have affixed my signature.

ALBERT L. CLAPP.